

## UNITED STATES PATENT OFFICE

2,322,307

## COMPOUNDED OIL

George L. Neely and Frank W. Kavanagh, Berkeley, Calif., assignors to Standard Oil Company of California, San Francisco, Calif., a corporation of Delaware

No Drawing. Application June 20, 1939,  
Serial No. 280,124

## 11 Claims. (Cl. 252—33)

The invention relates to compounded lubricating oils, and especially involves the provision of improved lubricating oils for internal combustion engines which will inhibit piston ring sticking and which will possess other advantageous properties not obtainable with prior known single compounding agents. Additionally, the invention provides lubricants having not only the ability to inhibit piston ring sticking but characterized by reduced corrosivity toward bearing metals, reduced jelling tendencies where jelling may not be desired, and enhanced lubrication values as indicated by factors such as improved ability to prevent scoring and uneven or undue wear of pistons, piston rings or cylinder walls of engines, and also as determined by ability to wet or adhere to hot metal surfaces, by lower wear, by lower friction and higher film strength, and by enhanced protection to bearings under high loads. The principles of this invention also permit production of compounded lubricants and compounding agents therefor having improved stability as respects resistance to oxidation, to high temperatures, to storage at low temperatures, and to storage in the presence of water.

The desirability of preventing the formation of adhesive oxidation products in hydrocarbons at elevated temperatures such as 425° to 525° F. has been recognized. In general, however, oxidation inhibitors which are operative at lower temperatures to inhibit the formation of such materials are not operative at extremely high temperatures, such as 500° F. Because of the inherent instability of hydrocarbons in the presence of an oxidizing agent under such extreme conditions of temperature, the possibility of finding a satisfactory oxidation inhibitor has not been promising, and there appears to be no known law of chemical nature which would enable one to predict or select from the vast list of chemical compounds those which would be operative at temperatures above 425° F. A large number of known oxidation inhibitors have been tried under these severe conditions and found to be unsatisfactory or totally inoperative.

When hydrocarbon compounds such as those occurring in mineral oils of the lubricating boiling range are heated to temperatures of from approximately 425° to 525° F. in the presence of an oxidizing agent such as an oxygen-containing gas, these compounds are partially oxidized and tend to deposit an adhesive gum or resinous material on surfaces with which they are in contact. Analysis of such deposits indicates that

the adhesive constituents comprise oxy or hydroxy organic acids and resinous complexes of these acids, which complexes are of unknown constitution and are apparently produced by further oxidation of the acids and/or by condensation as through inter-esterification of the hydroxy groups present therein.

It has been discovered that incorporation of certain metal salts of different organic acids in the hydrocarbon mixture will inhibit formation of an adhesive deposit on metal surfaces at elevated temperatures, although such salts may not prevent or inhibit partial oxidation and decomposition of the hydrocarbons. The formation of adhesive deposits is prevented by the metal salts altering the course of the oxy acid resinification reaction.

It is often found that salts in which the acid components consist entirely of one acid are not satisfactory compounding agents for lubricating oils, or at least do not possess other properties which are desirable or necessary in liquid lubricating compositions. These deficiencies may arise from unsatisfactory wear rate, instability of either the compounding agent or the compounded oil, or both, at high temperatures, instability of the oil solution of the compounding agent in storage or in the presence of water, undue corrosivity of the compounded oil toward bearing metals such as cadmium-silver or copper-lead alloys, unsatisfactory solubility of the compounding agent in the oil at low temperatures as indicated by cloud formation or jelling, undue foaming, unsatisfactory adhesion of the compounded oil to hot metal surfaces, and undesirably high friction or low film strength.

The present invention avoids at least part of the above difficulties by incorporating in the lubricating oil mixed organic salts of certain metals, said mixed salts containing different types of organic acids.

In producing the lubricating compositions of this invention, salts of metals selected from the group consisting of aluminum, calcium, barium, strontium, zinc, magnesium, cobalt, cadmium, manganese, tin and chromium may be utilized. Suitable mixtures and/or complex salts may be prepared by precipitation from aqueous solution. Thus one method comprises preparing an aqueous solution containing alkali metal salts of the mixture of acids in question, e. g. sodium naphthenate and sodium stearate, in substantially equal quantities, and then precipitating the polyvalent metal salts of these acids by adding a solution containing the appropriate metal ion,

e. g. an aqueous solution of aluminum sulfate. Such precipitation processes are preferably carried out in the presence of an organic solvent to take up the oil-soluble organic salt as it is formed. A suitable solvent comprises lubricating oil. It is to be understood that the invention, in its broader aspect, is not limited to salts prepared by simultaneous precipitation or by any other specific method.

To illustrate results which may be obtained by utilizing metal salts containing different types of organic acids, the following specific examples of lubrication problems involved and difficulties overcome are given:

Incorporation of both aluminum naphthenates and aluminum salts of long chain fatty acids in lubricating oils gives improvements in lubricants which are not attainable with either salt alone. For example, 1% aluminum stearate, when dissolved in a mineral oil lubricant, causes the formation of a jell and tends to separate from the oil at low temperatures. Such a lubricant is unsatisfactory for use in internal combustion engines. By contrast, addition of 0.5% aluminum naphthenate and 0.5% aluminum stearate (total aluminum salt content is still 1%) gives a liquid non-jelling lubricant, and the tendency of the aluminum stearate to precipitate out of the oil solution at low temperatures is avoided.

Furthermore, the lubricant containing aluminum naphthenate and aluminum stearate in combination not only possesses the ability to withstand severe high temperatures without depositing gum and carbon around the piston rings of an internal combustion engine but also gives superior protection to the Babbitt bearings of such engines. The following engine tests will illustrate this property of the oil.

#### Reduced area bearing tests

|                                                                                                               | Acid refined S. A. E. 30 Western oil+1% aluminum dinaphthenate + 0.25% stearic acid | Acid refined S. A. E. 30 Western oil+1/2% aluminum dinaphthenate+1/2% aluminum stearate |                 |                     |
|---------------------------------------------------------------------------------------------------------------|-------------------------------------------------------------------------------------|-----------------------------------------------------------------------------------------|-----------------|---------------------|
|                                                                                                               | Bearings tested                                                                     | Condition                                                                               | Bearings tested | Condition           |
| Single cylinder caterpillar engine 13 hour test. (Bearings out sway to increase unit load 230% above normal.) | 7                                                                                   | 6 failed (4 badly cracked).                                                             | 4               | 1 cracked slightly. |

It is to be noted that the above test is an extremely severe one and involves bearing loads not encountered in service. This test accentuates the ability of the lubricant to protect bearings under extreme conditions.

A second test illustrates performance of the same oil in protecting full size bearings in a 4-cylinder "RD-4" Caterpillar Diesel engine operating under severe conditions of full load and speed. The conditions of the test were: load, 75 lbs. B. M. E. P.; speed, 1400 R. P. M.; jacket temperature, 75° F.; oil temperature, 185° F. In this test there was no failure of any bearings after 541 hrs. of operation, whereas with a lubricant containing 1% aluminum dinaphthenate and 0.25% stearic acid failure of a bearing occasionally occurs under the severe conditions of the test after 200 hrs. operation.

Tests in which a single cylinder gasoline engine was operated under severe conditions designed to accelerate piston ring sticking show that an oil

containing 1/2% aluminum naphthenate and 1/2% aluminum stearate will inhibit piston ring sticking under such conditions for 120 hrs. or more of engine operation, whereas the same lubricating oil without the addition of the aluminum salts will permit piston ring sticking in 30 to 40 hrs.

The oil containing both aluminum dinaphthenate and aluminum stearate gives improved rates of wear over that obtained by the use of

10 aluminum dinaphthenate alone. A laboratory wear-testing machine comprising a 1/2 inch steel ball pressed against a 1 1/8 inch steel cylinder with a force of 40 lbs. and having the cylinder dipping in the oil to be tested and rotated at 600 R. P. M. for 16 hrs. was used to compare relative wear rates. Assuming the rate of wear to be 100% on this machine with an oil containing 1% aluminum dinaphthenate alone, an oil containing 1/2% aluminum stearate plus 1/2% aluminum dinaphthenate gives only 30% as much wear as the oil containing only aluminum naphthenate. This represents a reduction of 70% obtained by the use of the combination of salts of aluminum.

For purposes of illustration and to enable preparation of a lubricating oil according to the principles of this invention without unnecessary experimentation, the following example is given:

A basic aluminum naphthenate containing two equivalent weights of naphthenic acid to 30 three equivalent weights of aluminum is obtained by any of the well known methods. Naphthenic acids are generally prepared by extracting the naturally occurring naphthenic acids from crude petroleum oils or other distillates containing them, usually by washing the said oils with dilute aqueous caustic soda solution whereby water-soluble alkali naphthenates are formed. The alkali naphthenate solution may then be extracted with organic solvents to 40 remove the major proportion of inert mineral oil contained therein. The basic aluminum naphthenate may then be prepared by adding to a substantially neutral aqueous sodium naphthenate solution a caustic alkali and a water-soluble aluminum salt in proportions of one equivalent weight of hydroxide (OH) per three equivalent weights of aluminum. The water-insoluble basic aluminum naphthenate will be precipitated and the sodium salts will remain in solution. A mineral oil concentrate is prepared by dissolving ten parts by weight of the naphthenate in ninety parts by weight of the mineral oil. This concentrate is added to a mineral lubricating oil such as an S. A. E. 30 acid refined 50 naphthenic lubricating oil stock, in quantities sufficient to give 1% by weight of naphthenate based on the completed oil. This oil is then heated for about thirty minutes at a temperature of 250° F. by indirect heat. If superheated open steam is used for this heating operation a shorter time will generally suffice.

An equal portion of oil base is compounded with aluminum stearate by dissolving the stearate in oil in quantities sufficient to give a solution containing 1% aluminum stearate by weight. The oil containing the aluminum stearate is agitated thoroughly and heated to 65 350° F. until the salt is dissolved and the solution is clear. The batch may be heated in the presence of open steam until the viscosity at 210° F. is substantially equal to the viscosity of the original oil.

The two portions of oil, i. e. the one containing 1% aluminum dinaphthenate and the other 70 1% aluminum stearate, are mixed in equal pro-

portions at a temperature above 150° F. The aluminum stearate compounded portion preferably should not be allowed to cool after it has been prepared before mixing with the portion of oil compounded with the aluminum naphthenate.

The following further illustrates the advantages and effects which may be obtained by the use of complex or mixed salts prepared by precipitation from an aqueous solution containing water-soluble alkali salts of the corresponding acids. A mixed or complex aluminum stearate-naphthenate may be prepared by dissolving sodium naphthenate and sodium stearate in equal proportions in water and adding aluminum sulfate thereto until precipitation ceases. The following data are illustrative:

| Oil tested                                                                                            | Stability in storage at 32° F. | Wear              |
|-------------------------------------------------------------------------------------------------------|--------------------------------|-------------------|
| S. A. E. 30 acid refined naphthenic oil                                                               | Stable.....                    | 0.36.             |
| S. A. E. 30 acid refined naphthenic oil plus 1% aluminum dinaphthenate.                               | ... do .....                   | 1.40.             |
| S. A. E. 30 acid refined naphthenic oil plus 1% aluminum stearate.                                    | Separates .....                | Foams and scuffs. |
| S. A. E. 30 acid refined naphthenic oil plus 0.5% aluminum dinaphthenate.                             | Stable.....                    | 0.70.             |
| S. A. E. 30 acid refined naphthenic oil plus 0.5% aluminum stearate.                                  | Separates .....                | Foams and scuffs. |
| S. A. E. 30 acid refined naphthenic oil plus 0.5% aluminum dinaphthenate plus 0.5% aluminum stearate. | Stable.....                    | 0.40.             |

The procedure for determining the above data on wear is the same as previously described.

The above tests show that an oil containing aluminum stearate alone foams and scuffs in the wear test and that the compounding agent tends to separate at low temperatures. Likewise an oil containing aluminum dinaphthenate alone has a wear rate substantially higher than that of the corresponding uncompounded oil. When both compounding agents, prepared either by simultaneous or separate precipitation, are added to the lubricating oil the aluminum naphthenate component prevents the foaming and scuffing action obtained with aluminum stearate alone and maintains the stearate in solution at low temperatures. Also, the wear rate of the oil containing both aluminum dinaphthenate and aluminum stearate (total aluminum salt 1%) is 57% and 30% of the wear rate for the oils containing respectively 0.5% and 1% of aluminum dinaphthenate alone.

The relative proportions of naphthenate to stearate either in the complex or mixed salts may vary rather widely, depending upon the characteristics desired and the conditions to be encountered. In general, however, the proportion should range from four to six parts of the naphthenate to six to four parts of the stearate, respectively. Substantially equal parts of the stearate and naphthenate are preferred.

The invention is not limited to processes and compositions containing the above described specific complex or mixed salts but embraces liquid mineral oil compositions and processes of treating the same in which other mixed salts may be utilized. As has been previously stated, salts of the following metals are useful for the purposes of this invention: aluminum, calcium, barium, strontium, zinc, magnesium, cobalt, cadmium, manganese, tin and chromium. The invention embraces, for example, the following combinations or mixtures: saturated fatty acid-naphthenic acid salts, saturated fatty acid-phenate salts, saturated fatty acid-organo phosphoric

acid salts, saturated fatty acid-aromatic carboxylic acid salts, naphthenic acid-sulfonic acid salts, naphthenic acid-phenate salts, naphthenic acid-organo phosphoric acid salts, naphthenic acid-aromatic carboxylic acid salts, sulfonic acid-phenate salts, sulfonic acid-aromatic carboxylic acid salts, phenate-organo phosphoric acid salts, phenate-aromatic carboxylic acid salts.

- 10 Wherever used herein, the term "saturated fatty acids" designates saturated acids of the fatty acid series containing more than approximately ten carbon atoms and includes substituted fatty acids, such as phenyl stearic acid. Likewise, the 15 term "organo phosphoric acid" or "organo substituted acids of phosphorus" is utilized to designate acids of phosphorus containing an organic substituent.

Examples of saturated fatty acid-naphthenic acid mixed or complex salts are: aluminum stearate-naphthenate, calcium stearate-naphthenate, zinc stearate-naphthenate, magnesium stearate-naphthenate, cobalt stearate-naphthenate, cadmium stearate-naphthenate, manganese stearate-naphthenate, tin stearate-naphthenate, and chromium stearate-naphthenate.

Examples of saturated fatty acid-sulfonic acid mixed or complex salts are: aluminum stearate-cetyl anthracene sulfonate, calcium stearate-cetyl anthracene sulfonate, zinc stearate-cetyl anthracene sulfonate, magnesium stearate-cetyl anthracene sulfonate, cobalt stearate-cetyl anthracene sulfonate, cadmium stearate-cetyl anthracene sulfonate, manganese stearate-cetyl anthracene sulfonate, tin stearate-cetyl anthracene sulfonate, and chromium stearate-cetyl anthracene sulfonate.

Examples of saturated fatty acid-phenate mixed or complex salts are: aluminum stearate-cetyl phenate, calcium stearate-cetyl phenate, zinc stearate-cetyl phenate, magnesium stearate-cetyl phenate, cobalt stearate-cetyl phenate, cadmium stearate-cetyl phenate, manganese stearate-cetyl phenate, tin stearate-cetyl phenate, and chromium stearate-cetyl phenate.

Examples of saturated fatty acid-organo phosphoric acid mixed or complex salts are: aluminum phenyl stearate-cetyl phosphate, calcium phenyl stearate-cetyl phosphate, zinc phenyl stearate-cetyl phosphate, magnesium phenyl stearate-cetyl phosphate, cobalt phenyl stearate-cetyl phosphate, cadmium phenyl stearate-cetyl phosphate, manganese phenyl stearate-cetyl phosphate, tin phenyl stearate-cetyl phosphate, and chromium phenyl stearate-cetyl phosphate.

Examples of saturated fatty acid-aromatic carboxylic acid mixed or complex salts are: aluminum stearate-cetyl benzoate, calcium stearate-cetyl benzoate, zinc stearate-cetyl benzoate, magnesium stearate-cetyl benzoate, cobalt stearate-cetyl benzoate, manganese stearate-cetyl benzoate, tin stearate-cetyl benzoate, and chromium stearate-cetyl benzoate.

Examples of naphthenic acid-sulfonic acid mixed or complex salts are: aluminum naphthenate-cetyl anthracene sulfonate, calcium naphthenate-cetyl anthracene sulfonate, zinc naphthenate-cetyl anthracene sulfonate, magnesium naphthenate-cetyl anthracene sulfonate, cobalt naphthenate-cetyl anthracene sulfonate, cadmium naphthenate-cetyl anthracene sulfonate, manganese naphthenate-cetyl anthracene sulfonate, tin naphthenate-cetyl anthracene sul-

fonate, and chromium naphthenate-cetyl anthracene sulfonate.

Examples of naphthenic acid-phenate mixed or complex salts are: aluminum naphthenate-cetyl phenate, calcium naphthenate-cetyl phenate, zinc naphthenate-cetyl phenate, magnesium naphthenate-cetyl phenate, cobalt naphthenate-cetyl phenate, cadmium naphthenate-cetyl phenate, manganese naphthenate-cetyl phenate, tin naphthenate-cetyl phenate, and chromium naphthenate-cetyl phenate.

Examples of naphthenic acid-organo phosphoric acid mixed or complex salts are: aluminum naphthenate-cetyl phosphate, calcium naphthenate-cetyl phosphate, zinc naphthenate-cetyl phosphate, magnesium naphthenate-cetyl phosphate, cobalt naphthenate-cetyl phosphate, cadmium naphthenate-cetyl phosphate, manganese naphthenate-cetyl phosphate, tin naphthenate-cetyl phosphate, and chromium naphthenate-cetyl phosphate.

Examples of naphthenic acid-aromatic carboxylic acid mixed or complex salts are: aluminum naphthenate-cetyl benzoate, calcium naphthenate-cetyl benzoate, zinc naphthenate-cetyl benzoate, magnesium naphthenate-cetyl benzoate, cobalt naphthenate-cetyl benzoate, cadmium naphthenate-cetyl benzoate, manganese naphthenate-cetyl benzoate, tin naphthenate-cetyl benzoate, and chromium naphthenate-cetyl benzoate.

Examples of sulfonic acid-phenate mixed or complex salts are: aluminum cetyl phenate-petroleum sulfonate, calcium cetyl phenate-petroleum sulfonate, zinc cetyl phenate-petroleum sulfonate, magnesium cetyl phenate-petroleum sulfonate, cobalt cetyl phenate-petroleum sulfonate, cadmium cetyl phenate-petroleum sulfonate, manganese cetyl phenate-petroleum sulfonate, tin cetyl phenate-petroleum sulfonate, chromium cetyl phenate-petroleum sulfonate, aluminum cetyl phenate-cetyl anthracene sulfonate, calcium cetyl phenate-cetyl anthracene sulfonate, zinc cetyl phenate-cetyl anthracene sulfonate, magnesium cetyl phenate-cetyl anthracene sulfonate, cobalt cetyl phenate-cetyl anthracene sulfonate, cadmium cetyl phenate-cetyl anthracene sulfonate, manganese cetyl phenate-cetyl anthracene sulfonate, tin cetyl phenate-cetyl anthracene sulfonate, and chromium cetyl phenate-cetyl anthracene sulfonate.

Examples of sulfonic acid-organo phosphoric acid mixed or complex salts are: aluminum cetyl phosphate-petroleum sulfonate, calcium cetyl phosphate-petroleum sulfonate, zinc cetyl phosphate-petroleum sulfonate, magnesium cetyl phosphate-petroleum sulfonate, cobalt cetyl phosphate-petroleum sulfonate, cadmium cetyl phosphate-petroleum sulfonate, manganese cetyl phosphate-petroleum sulfonate, tin cetyl phosphate-petroleum sulfonate, chromium cetyl phosphate-petroleum sulfonate, aluminum cetyl phosphate-cetyl anthracene sulfonate, calcium cetyl phosphate-cetyl anthracene sulfonate, zinc cetyl phosphate-cetyl anthracene sulfonate, magnesium cetyl phosphate-cetyl anthracene sulfonate, cobalt cetyl phosphate-cetyl anthracene sulfonate, cadmium cetyl phosphate-cetyl anthracene sulfonate, manganese cetyl phosphate-cetyl anthracene sulfonate, tin cetyl phosphate-cetyl anthracene sulfonate, and chromium cetyl phosphate-cetyl anthracene sulfonate.

Examples of sulfonic acid-aromatic carboxylic acid mixed or complex salts are: aluminum cetyl benzoate-petroleum sulfonate, calcium cetyl

benzoate-petroleum sulfonate, zinc cetyl benzoate-petroleum sulfonate, magnesium cetyl benzoate-petroleum sulfonate, cobalt cetyl benzoate-petroleum sulfonate, cadmium cetyl benzoate-petroleum sulfonate, manganese cetyl benzoate-petroleum sulfonate, tin cetyl benzoate-petroleum sulfonate, chromium cetyl benzoate-petroleum sulfonate, aluminum cetyl benzoate-cetyl anthracene sulfonate, calcium cetyl benzoate-cetyl anthracene sulfonate, zinc cetyl benzoate-cetyl anthracene sulfonate, magnesium cetyl benzoate-cetyl anthracene sulfonate, cobalt cetyl benzoate-cetyl anthracene sulfonate, cadmium cetyl benzoate-cetyl anthracene sulfonate, manganese cetyl benzoate-cetyl anthracene sulfonate, tin cetyl benzoate-cetyl anthracene sulfonate, and chromium cetyl benzoate-cetyl anthracene sulfonate.

Examples of phenate-organo phosphoric acid mixed or complex salts are: aluminum cetyl phenate-cetyl phosphate, calcium cetyl phenate-cetyl phosphate, zinc cetyl phenate-cetyl phosphate, magnesium cetyl phenate-cetyl phosphate, cobalt cetyl phenate-cetyl phosphate, cadmium cetyl phenate-cetyl phosphate, manganese cetyl phenate-cetyl phosphate, tin cetyl phenate-cetyl phosphate, and chromium cetyl phenate-cetyl phosphate.

Examples of phenate-aromatic carboxylic acid mixed or complex salts are: aluminum cetyl phenate-cetyl benzoate, calcium cetyl phenate-cetyl benzoate, zinc cetyl phenate-cetyl benzoate, magnesium cetyl phenate-cetyl benzoate, cobalt cetyl phenate-cetyl benzoate, cadmium cetyl phenate-cetyl benzoate, manganese cetyl phenate-cetyl benzoate, tin cetyl phenate-cetyl benzoate, and chromium cetyl phenate-cetyl benzoate.

The combinations herein disclosed yield lubricants having improved characteristics which are not obtainable with metal salts having single organic acid components. In general, the combinations of this invention cooperate to give lubricants having one or more improved characteristics as compared with lubricants using the single elements of the combinations. For example, mixed salts having a fatty acid component give improved lubrication value or resistance to wear and enhanced protection of bearings operating under severe conditions. Combinations containing phenate components have lower corrosion and greater stability at elevated temperatures than do oils containing a fatty acid salt alone, for instance. Also, the phenate components increase the stability of the oil solution of the fatty acid salts and the like. The organo phosphoric acid component increases the stability of the oil to high temperatures and its resistance to oxidation, as well as improves wetting and adhesion characteristics of the oil to hot metallic surfaces. This component also reduces the corrosivity of the oils toward copper-lead or cadmium-silver bearing metal alloys. Certain of the sulfonates reduce friction, corrosion, and enhance oxidation stability of particular combinations. The phenates and sulfonates tend to reduce jell-formation of other components of the combinations in certain instances.

The phenates used in the combinations of this invention are preferably high molecular weight compounds in which the phenolic radical contains at least eleven carbon atoms. The organo phosphate compounds are also preferably high molecular weight materials in which the acid of

phosphorus contains an organic substituent having at least twelve carbon atoms. It should be observed that the invention, in its broader aspects, is not limited to substituted phosphoric acids but includes other substituted acids of phosphorus, such as phosphorous acid, as well as other substituted acids of pentavalent phosphorus.

The proportion of metal salts added to the hydrocarbon mixtures may vary widely, depending upon the salt selected and the conditions to be encountered. The present invention is primarily concerned with the production of liquid hydrocarbon compositions and the proportion of the metal salts should therefore preferably be insufficient to solidify the hydrocarbon mixture. In general, it has been found that from approximately 0.5% to approximately 2% of total salt content, based on the weight of the hydrocarbons, serve the purposes of the invention although as little as 0.1% or as much as 5% is not precluded. The metal salts may be incorporated in high boiling hydrocarbons of widely different types. Hydrocarbons of petroleum origin are the most commonly available and will be most generally utilized. Pennsylvania, Mid-Continent or California petroleums are suitable sources for high boiling hydrocarbons of the type here involved. Although paraffinic oils such as commonly obtained from Pennsylvania crudes are not precluded, it has been found that acid refined naphthenic base oils are more readily susceptible to improvement as respects formation of adhesive resinous deposits on metal surfaces at elevated temperature. Synthetic hydrocarbons, for example, olefin hydrogenated polymers such as butene, isobutene or mixed butene hydrogenated polymers, may be utilized. In general, the hydrocarbon should be of a liquid consistency at ordinary atmospheric temperatures and should preferably have a boiling point above approximately 500° F. at atmospheric pressure.

The relative proportion of the respective acid components in the complex or mixed salts contained in the compounded lubricating oils herein disclosed will vary, depending upon the purposes to be served and conditions encountered during use. In general, the ratio of acid components will be no greater than ten to one, and preferably will be from approximately four to one, on the one hand, to one to one, on the other hand—these being stoichiometrical proportions.

The compositions of this invention have a number of applications and will be found to have utility where it is desirable to inhibit deposition and/or formation of adhesive gums on metal surfaces which are bathed in or are in contact with high boiling hydrocarbons subjected to elevated temperatures in the presence of an oxidizing agent such as an oxygen-containing gas. One example of such an application comprises the lubrication of Diesel engines in which the oil is spread in a thin film over the pistons, piston rings and cylinder walls of the engine, and is subjected to the oxidizing action of the compressed gases in the combustion chamber at temperatures of from approximately 425° to 525° F. or above which exist at the upper piston rings of such engines. In this particular application of the invention it should be noted that the hydrocarbons are subjected not only to high temperatures in thin films on the metal surfaces, but also to the high pressures necessary to produce spontaneous ignition of Diesel fuels. These pressures are approximately 400 to 600 lbs./sq. in. at the time of ignition of the fuel, and rise to pres-

sures as high as 750 to 1150 lbs./sq. in. during combustion of the fuel. By the present process the normal course of reactions occurring in the oil under these conditions may be progressively altered so that formation and/or deposition of adhesive materials is prevented and piston ring sticking is inhibited.

The compositions of this invention are also applicable to the prevention of formation and/or deposition of adhesive materials from hydrocarbon mixtures in those various instances where an oil flows over a metal surface which is heated to high temperatures and where heat transfer is the primary object to be accomplished. For example, oil cooled electric resistances subject the oil to high temperatures at the oil-metal interface of the highly heated electric resistance element. The deposition of adhesive gummy materials on the surface of the resistance element may be inhibited at temperatures as high as 425° to 525° F. and the efficiency of the heat transfer thereby maintained or increased. An oxidizing agent will generally be present in such heat transfer process by reason of dissolved oxygen which is contained in the oil being heated, as well as by reason of air which may be in contact with the oil at one or more points in the system.

The compounding agents herein disclosed may have one or more advantages depending upon the particular compounds selected, the proportion utilized, and the environment which the compounded oil is to encounter. It should be observed, for example, that even though a compounded oil may be somewhat corrosive to copper-lead or cadmium-silver bearing metals, Babbitt bearings are little if at all affected by such corrosive action at temperatures where they are not unsatisfactory for other reasons, such as low melting point or lack of fatigue resistance. Hence, compounded oils which may not be particularly desirable for lubrication of copper-lead or cadmium-silver bearings may be highly useful and extremely advantageous in conjunction with the operation of internal combustion engines having bearings of Babbitt or other corrosion-resistant bearing metals. The present invention, in its broader aspects, is therefore not limited to combinations having all or the greatest number of advantages, but embraces various of the less advantageous combinations which will find utility in particular applications where all the possible improvement in properties may not be required or where the standard of performance may not be so high.

The mixed salts of this invention may be added to hydrocarbon oils containing other compounding ingredients, such as pour point depressors, blooming agents, compounds for enhancing the viscosity index of the hydrocarbon oil, etc. The invention in its broader aspects embraces hydrocarbon oils containing, in addition to the mixed salts herein disclosed, thickening agents in grease-forming proportions or in amounts insufficient to form greases, as in the case of mineral castor machine oils or other compounded liquid lubricants.

A part of the subject matter of this application is disclosed in the original specification of applicants' earlier application Serial No. 62,814 now issued as Patent No. 2,163,622 of June 26, 1939, on Compounded lubricating oil. This common subject matter was divided out of parent case No. 62,814 for inclusion in the present application.

Our copending application Serial No. 476,056,

filed February 16, 1943, is directed to those aspects of the invention relating to the combination of sulfonates and organo-phosphates and to the combination of sulfonates and naphthenates or aromatic carboxylates.

While the character of this invention has been described in detail and numerous illustrations given, this has been done with the intention that no limitation should be imposed upon the invention thereby. It will be apparent to those skilled in the art that numerous modifications and variations of the above disclosures may be effected in the practice of the invention which is of the scope of the claims appended hereto.

We claim:

1. A compounded liquid lubricant comprising a liquid hydrocarbon oil subject to deterioration and deposition of adhesive materials at elevated temperatures, said hydrocarbon oil containing from approximately 0.1% to approximately 5% by weight based on the oil of oil-soluble mixed salts of aluminum having a naphthenic and a saturated higher fatty acid radical, said mixed salts being present in an amount sufficient substantially to reduce said deposition.

2. A compounded liquid lubricant comprising a liquid hydrocarbon oil subject to deterioration and deposition of adhesive materials at elevated temperatures, said hydrocarbon oil containing, in an amount sufficient substantially to reduce said deposition, oil-soluble mixed salts of aluminum having as one radical a high molecular weight phenate radical.

3. A compounded liquid lubricant comprising a liquid hydrocarbon oil subject to deterioration and deposition of adhesive materials at elevated temperatures, said hydrocarbon oil containing, in an amount sufficient substantially to reduce said deposition, oil-soluble mixed salts of aluminum having as one component a radical of a high molecular weight substituted acid of phosphorus containing an organic substituent.

4. A compounded liquid lubricant comprising a liquid hydrocarbon oil subject to deterioration and deposition of adhesive materials at elevated temperatures, said hydrocarbon oil containing, in an amount sufficient substantially to reduce said deposition, oil-soluble mixed salts of aluminum having a sulfonate and a phenate radical.

5. A compounded liquid lubricant comprising a liquid hydrocarbon oil subject to deterioration and deposition of adhesive materials at elevated temperatures, said hydrocarbon oil containing, in an amount sufficient substantially to reduce said deposition, oil-soluble complex salts of a polyvalent metal and having as one component a high molecular weight phenate radical.

6. A compounded liquid lubricant comprising a liquid hydrocarbon oil subject to deterioration and deposition of adhesive materials at elevated temperatures, said hydrocarbon oil containing, in an amount sufficient substantially to reduce said deposition, oil-soluble complex salts of a polyvalent metal and having as one component a radical of a substituted acid of phosphorus containing an organic substituent.

7. A compounded liquid lubricant comprising a liquid hydrocarbon oil subject to deterioration and deposition of adhesive materials at elevated temperatures, said hydrocarbon oil containing, in an amount sufficient substantially to reduce said deposition, oil-soluble mixed polyvalent metal salts having a sulfonate and a phenate radical.

8. A compounded liquid lubricant comprising a liquid hydrocarbon oil subject to deterioration and deposition of adhesive materials at elevated temperatures, said hydrocarbon oil containing, in an amount sufficient substantially to reduce said deposition, oil-soluble mixed salts selected from the group consisting of aluminum, calcium, barium, strontium, zinc, magnesium, cobalt, cadmium, manganese, tin and chromium salts containing a naphthenic and a saturated higher fatty acid radical.

9. A compounded liquid lubricant comprising a liquid hydrocarbon oil subject to deterioration at elevated temperatures, said hydrocarbon oil containing in an amount sufficient substantially to reduce said deterioration, oil-soluble mixed salts of a polyvalent metal, said mixed salts having as salt-forming acid radicals a substituted acid of phosphorus containing an organic substituent and an organic carboxylic acid containing an aryl substituent.

10. A compounded liquid lubricant comprising a liquid hydrocarbon oil subject to deterioration and deposition of adhesive materials at elevated temperatures, said hydrocarbon oil containing, in an amount sufficient substantially to reduce said deposition, oil-soluble mixed salts of aluminum having an alkaryl sulfonate and a phenate radical.

11. A compounded liquid lubricant comprising a liquid hydrocarbon oil subject to deterioration and deposition of adhesive materials at elevated temperatures, said hydrocarbon oil containing, in an amount sufficient substantially to reduce said deposition, oil-soluble mixed polyvalent metal salts having an alkaryl sulfonate and a phenate radical.

GEORGE L. NEELY,  
FRANK W. KAVANAGH.